

May 18, 1937.

H. K. WEICHMANN

2,080,551

SENSITIZING SILVER HALIDE EMULSION

Filed July 31, 1934

Fig. 1



Fig. 2



Fig. 3



Fig. 4



Fig. 5



Fig. 6



Fig. 7



## UNITED STATES PATENT OFFICE

2,080,551

## SENSITIZING SILVER HALIDE EMULSION

Hans Konrad Weichmann, Dessau in Anhalt,  
Germany, assignor to Agfa Ansco Corporation,  
Binghamton, N. Y., a corporation of New York

Application July 31, 1934, Serial No. 737,853  
In Germany August 3, 1933

5 Claims. (Cl. 95—7)

My present invention relates to sensitizing silver halide emulsions.

One of its objects is a silver halide emulsion which has been rendered sensitive to waves for which the emulsion is normally not sensitive. 5 Further objects will be seen from the detailed specification following hereafter.

In the accompanying drawing there have been shown spectrograms of silver halide emulsions according to this invention in comparison with a not 10 specially sensitized emulsion and an emulsion containing a known sensitizer.

It has already been proposed to sensitize a silver halide emulsion by the incorporation of a 15 benzoxo-indo-trimethinecyanine which is not substituted in the benzene nuclei. The emulsions thus sensitized are not suited for the production of orthochromatic emulsions of a very high sensitivity inasmuch as the sensitizing power of these 20 benzoxo trimethinecyanines is, for instance, not greater than that of erythrosine. Furthermore the range of sensitivity reaches only from the initial sensitivity to about 590  $\mu\mu$ .

I have found that a silver halide emulsion sensitized with a benzoxo-indo-trimethinecyanine 25 which has been substituted preferably by an alkoxy group or an alkyl group or both in one or both benzene nuclei yields an orthochromatic emulsion of highest sensitivity. The sensitivity of 30 the emulsions is greater than that obtained with the use of the hitherto known sensitizers.

The sensitizing dyes may be obtained by condensing a quaternary ammonium salt of a benzoxazole or an indole with di-phenylformamidine 35 in the presence of acetic anhydride to form an intermediate product and condensing the intermediate product with the desired indolenine or benzoxazole respectively in the presence of pyridine, or the dyes may be made by condensing an 40 indolenine compound containing in  $\alpha$ -position to the nitrogen atom a methylene group capable of reaction of which one hydrogen atom has been substituted by the aldehyde group with a quaternary ammonium salt of a benzoxazole in solvents 45 such as pyridine, nitrobenzene, acetic anhydride, and in the presence of a condensing agent, for instance, phosphoroxychloride or piperidine.

By sensitizing a silver halide emulsion with a sensitizing agent according to this invention the sensitivity to green and yellow and simultaneously 50 the total sensitivity is increased and in consequence a better rendition of the colors is obtained without affecting the possibility to develop the exposed emulsion in red light.

55 The spectrograms of the accompanying drawing show the high sensitivity which lies in a spectral region as it is desired, and it can easily be recognized that the unsubstituted benzoxo-indolenine-trimethinecyanines have a much less intense sensitizing effect.

Figure 1 shows an unsensitized silver bromide emulsion, containing about 4 per cent of silver iodide.

Figure 2 shows the same silver bromide emulsion sensitized with the most favorable amount 5 of the unsubstituted benzoxo-indolenine-trimethinecyanine.

Figure 3 shows the same silver bromide emulsion sensitized with [3-ethyl-6-methoxy-benzoxazole(2) 1-[1.dimethyl-3-methyl-indolenine(2) 10 trimethinecyanine iodide,

Figure 4 shows the same silver bromide emulsion sensitized with [3-ethyl-benzoxazole(2) 1-[1.dimethyl-3.5.6.trimethyl-indolenine(2) 15 trimethinecyanine perchlorate,

Figure 5 shows the same silver bromide emulsion sensitized with [3.5.6.trimethyl-benzoxazole(2) 1-[1.dimethyl-3.6.dimethyl-indolenine(2) 20 trimethinecyanine iodide,

Figure 6 shows the same silver bromide emulsion sensitized with [3-ethyl-6.methoxy-benzoxazole(2) 1-[1.dimethyl-3.6.dimethyl-indolenine(2) 25 trimethinecyanine iodide,

Figure 7 shows the same silver bromide emulsion sensitized with [3.5.6.trimethyl-benzoxazole(2) 30 1-[1.dimethyl-3.5.6.trimethyl-indolenine(2) 35 trimethinecyanine iodide.

The dyes are obtainable according to the desired solubility in form of the bromide, iodide, perchlorate etc. and are used in a quantity, such as is usual for the known sensitizing dyes. This quantity may amount to about 10 to 30 milligrams per kilo of emulsion ready for being cast which contains about 9 per cent of gelatin, 4.5 per cent of silver halide and the rest water. However, the invention is not limited to the quantities just indicated and the most suitable amount can be found in each case by a few comparative experiments. The dyes may be added to the emulsion in form of solutions. Suitable solvents are the alcohols, for instance, methyl or ethyl alcohol which may be used anhydrous or diluted with water. The dyes are applied to the emulsion during any stage of its production; however, they are preferably added to the finished emulsion 40 before casting.

The dyes may likewise be incorporated in the emulsion by coating the cast, but not dried, emulsion layer with a solution of the sensitizer in, for instance, aqueous or non-aqueous methyl alcohol 45 or ethyl alcohol, applied by means of a coating roller. The concentration of the solution depends upon the speed of coating; for example, when the speed of coating amounts to 20 cm. per second, a suitable solution may consist of about 1 mgr. of the sensitizer dissolved in 50 cc. of aqueous methyl alcohol of 50 per cent strength. Another method of incorporating the sensitizer in the emulsion consists in bathing the finished photographic material in a bath in which the dye is dissolved, 50 55 60

for instance, in a solution of methanol of 50 per cent strength containing 1 mgr. of dye in 50 cc. of aqueous methanol.

The oxazole bases may be obtained by distilling 5 the suitably substituted o-aminophenol with acetic anhydride. At first water distills over and at a temperature above 200° C. the benzoxazole.

The following examples illustrate the invention.

*Example 1.*—2-methyl-6-methoxybenzoxazole 10 is made by distilling the correspondingly substituted o-aminophenol with acetic anhydride. The compound distills over at a temperature above 200° C.

2-methyl-6-methoxybenzoxazole ethiodide is 15 made by heating 15.6 grams of ethyliodide and 16.3 grams of 2-methyl-6-methoxybenzoxazole for about 6 to 8 hours on the steam bath. The compound separates in the form of white needles.

5 grams of 2-methyl-6-methoxybenzoxazole 20 with 3 grams of diphenylformamidine and 16 cc. of acetic anhydride are boiled for about 5 minutes. After cooling the formed intermediate product is precipitated with ether and purified by washing with acetone. It is obtained in the form 25 of a yellow powder.

The dye [3-ethyl-6-methoxybenzoxazole (2)]-[1-dimethyl-3-methyl-indolenine (2)] trimethinecyanine iodide corresponding with the formula



30 is produced by heating a mixture of 4 grams of the above intermediate product, 3 grams of 1.1.2.3-tetramethylindolenine and 15 cc. of pyridine for about 2 hours to 135° C. After cooling, the dye 35 is precipitated by means of a 10 per cent aqueous solution of potassium iodide. The dye is purified by recrystallization from alcohol and is obtained in the form of a red powder.

The alcoholic solution of the dye has an absorption 40 maximum at a wave length of about 523  $\mu\mu$ .

Incorporated in a silver bromide emulsion containing about 4 per cent of silver iodide, the dye 45 imparts to it a range of sensitivity from about 500 to 610  $\mu\mu$  with a maximum at about 570  $\mu\mu$ .

*Example 2.*—2-methylbenzoxazole-p-toluenesulfoethylate is made by distilling o-aminophenol and acetic anhydride, and heating the 2-methylbenzoxazole obtained for about 8 hours to 140° C. with the equimolecular proportion of the ethyl ester of  $\beta$ -toluenesulfonic acid. The compound is 50 washed with acetone and forms white crystals.

4 grams of 2-methylbenzoxazole-p-toluenesulfoethylate and 3.5 grams of diphenylformamidine are boiled with 15 cc. of glacial acetic acid. After 55 cooling the intermediate product crystallizes in the form of needles on the addition of ether.

The dye [1-ethyl-benzoxazole (2)]-[1.dimethyl-3.5.6 trimethyl-indolenine (2)] trimethinecyanine perchlorate corresponding with the formula



60 is produced by heating 5 grams of 1.1.2.3.5.6-hexamethyl-indolenine methiodide and 4 grams of the above intermediate product with 15 cc. of pyridine for about 2 hours to 135° C. The mix-

ture assumes a red color and, after cooling the dye is precipitated by the addition of 5 cc. of a concentrated solution of sodium perchlorate. The perchlorate forms red needles which are recrystallized from alcohol.

The alcoholic solution of the dye has an absorption maximum at a wave length of about 522  $\mu\mu$ .

Incorporated in a silver bromide emulsion containing about 4 per cent. of silver iodide, the dye 10 imparts to it a range of sensitivity from about 500 to 615  $\mu\mu$  with a maximum at about 570  $\mu\mu$ .

*Example 3.*—12 grams of methyl-formaniline is mixed with 15 grams of phosphorus oxychloride while stirring at room temperature. Stirring is continued for about 2 hours, then the mixture is diluted with 15 grams of o-dichlorobenzene, cooled to 5° C., and mixed at this temperature with 17 grams of 1.1.3.6-tetramethyl-2-methylindolenine. After about 15 hours the mixture is distilled with steam and the non-volatile residue is, after drying, recrystallized from ligroin. The aldehyde crystallizes in the form of light-colored crystals.

3 grams of 2.5.6-trimethylbenzoxazole dimethylsulfate which is produced analogously to the other quaternary ammonium salts of benzoxazole and 2 grams of 1.1.3.5-tetramethylindolenine-2-methylene- $\omega$ -aldehyde are boiled with 10 cc. of pyridine for about 1.5 hours. Then there are added 5 cc. of a 10 per cent solution of potassium iodide. The red dye which corresponds with the formula



35 is precipitated in cooling and is recrystallized from alcohol.

The alcoholic solution of the dye has an absorption maximum at a wave length of about 525  $\mu\mu$ .

Incorporated in a silver bromide emulsion containing about 4 per cent. of silver iodide, the dye 45 imparts to it a range of sensitivity from about 500 to 615  $\mu\mu$  with a maximum at about 565  $\mu\mu$ .

*Example 4.*—The dye [3-ethyl-6-methoxybenzoxazole (2)]-[1-dimethyl-3.5.6-dimethyl-indolenine (2)] trimethinecyanine iodide corresponding with the formula



55 is produced by boiling 3 grams of 2-methyl-6-methoxybenzoxazole ethiodide (see Example 1) 60 and 2 grams of the intermediate product described in Example 3 with 7 cc. of pyridine for about 2 hours. After cooling the red dye is precipitated with a solution of potassium iodide and recrystallized from alcohol.

The alcoholic solution of the dye has an absorption maximum at a wave length of about 527  $\mu\mu$ .

Incorporated in a silver bromide emulsion containing about 4 per cent. of silver iodide, the dye 70 imparts to it a range of sensitivity from about 500 to 615  $\mu\mu$  with a maximum at about 572  $\mu\mu$ .

*Example 5.*—For producing 1.1.3.5.6-penta-methyl indolenine-2-methylene- $\omega$ -aldehyde, 12 grams of methylformaniline and 15 grams of sulfonylchloride are mixed and stirred for about 2 75

hours. After diluting with 15 grams of dichlorobenzene and cooling to 5° C. there are slowly added 18 grams of 1.1.3.5.6-pentamethyl-2-methyl indolenine while cooling. After about 15 hours 5 the mixture is distilled with steam and worked up as described in Example 3, whereby the aldehyde is obtained in the form of crystals.

The dye [3.5.6. trimethyl-benzoxazole (2)]-[1.dimethyl-3.5.6-trimethyl-indolenine (2)] trimethinecyanine iodide corresponding with the formula



15 is produced by boiling 2 grams of the above intermediate product and 3 grams of 2.5.6-trimethylbenzoxazole dimethylsulfate (see Example 2) with 15 cc. of pyridine at 135° C. for about 2 hours. On cooling the dye separates in the form 20 of crystals.

25 The alcoholic solution of the dye has an absorption maximum at a wave length of about 529  $\mu\mu$ .

Incorporated in a silver bromide emulsion con-

taining about 4 per cent of silver iodide, the dye imparts to it a range of sensitivity from about 500 to 618  $\mu\mu$  with a maximum at about 575  $\mu\mu$ .

What I claim is:

1. A photographic material comprising a silver halide emulsion containing a 3.3'-dialkyl-benzoxo-indolenine-trimethinecyanine salt containing in one of the benzene nuclei a substituent of the group consisting of alkyl and alkoxy.

10 2. A photographic material comprising a silver halide emulsion containing a 3.3'-dialkyl-benzoxo-indolenine-trimethinecyanine salt containing in both benzene nuclei a substituent of the group consisting of alkyl and alkoxy.

15 3. A photographic material comprising a silver halide emulsion containing [3-ethyl-6-methoxy-benzoxazole (2)]-[1-dimethyl-3.6-dimethyl-indolenine (2)]-trimethinecyanine iodide.

20 4. A photographic material comprising a silver halide emulsion containing [3.5.6-trimethyl-benzoxazole (2)]-[1-dimethyl-3.6.dimethyl-indolenine (2)] trimethinecyanine iodide.

25 5. A photographic material comprising a silver halide emulsion containing [3.5.6.trimethyl-benzoxazole (2)]-[1-dimethyl-3.5.6-trimethyl-indolenine (2)] trimethinecyanine iodide.

HANS KONRAD WEICHMANN.